

# United States Patent Office.

WILLIAM ADAMSON, OF PHILADELPHIA, PENNSYLVANIA

*Letters Patent No. 65,787, dated June 18, 1867.*

## IMPROVEMENT IN THE MANUFACTURE OF GLUE.

The Schedule referred to in these Letters Patent and making part of the same.

### TO ALL WHOM IT MAY CONCERN:

Be it known that I, WILLIAM ADAMSON, of Philadelphia, Pennsylvania, have invented an improved Glue; and I do hereby declare the following to be a full, clear, and exact description of the same.

My invention consists of ordinary glue (or size prior to its conversion into glue) combined with borate of soda or borax, substantially as described hereafter, the product being a tenacious glue, partially bleached, and not so liable to fermentation and rotting as ordinary glue.

In order to enable others familiar with processes of this class to make my invention, I will now proceed to describe the mode of producing the same.

My invention may be carried into effect either by mixing dissolved glue with the borate of soda, or by mixing the latter with size prior to the conversion of the same into glue by the ordinary process of drying or desiccating, or by the aerating or carbonating process described in a separate application for a patent which I have this day made. The product may be obtained by dissolving about twenty pounds of borate of soda in as much water as will be necessary to effect a thorough solution, and mixing the latter with about one thousand pounds of melted glue or size. The proportion of the borax to the glue or size, however, will depend upon the condition of the latter, which condition can be readily understood and ascertained by those familiar with the manufacture of glue.

The solution of borate of soda may be applied in about the above proportions to size, prior to the conversion of the same into glue by the ordinary drying or desiccating process; but I prefer to apply the solution to the size immediately after aerating or treating the same with gas, as I have described in a separate application for a patent.

I claim as my invention, and desire to secure by Letters Patent—

The combination, substantially as described, of glue or size with borate of soda, for the purpose specified. In testimony whereof I have signed my name to this specification in the presence of two subscribing witnesses.

WM. ADAMSON.

Witnesses:

JOHN WHITE,  
W. J. R. DELANY.